

# United States Patent [19]

Johnson

[11] Patent Number: 4,532,760

[45] Date of Patent: Aug. 6, 1985

[54] D. C. YARN TENSION CONTROL

[75] Inventor: Harold L. Johnson, Pauline, S.C.

[73] Assignee: Milliken Research Corporation,  
Spartanburg, S.C.

[21] Appl. No.: 582,044

[22] Filed: Feb. 21, 1984

[51] Int. Cl.<sup>3</sup> D02G 3/34; D01H 13/10;  
B65H 59/22

[52] U.S. Cl. 57/283; 57/91;  
57/284; 57/287; 57/352

[58] Field of Search 57/90-94,  
57/100, 127.5, 127.7, 264, 282, 283, 284, 287,  
351, 352, 354

## [56] References Cited

### U.S. PATENT DOCUMENTS

|           |         |                  |           |
|-----------|---------|------------------|-----------|
| 2,624,527 | 1/1953  | Von Kohorn       | 242/155   |
| 2,705,362 | 4/1955  | Roughsedge       | 28/51     |
| 2,724,065 | 11/1955 | Saxl             | 310/93    |
| 2,931,090 | 4/1960  | Field, Jr.       | 28/1      |
| 2,946,177 | 7/1960  | Scragg et al.    | 57/284    |
| 2,978,203 | 4/1961  | Westall et al.   | 242/155   |
| 2,999,351 | 9/1961  | Davenport et al. | 57/140    |
| 3,011,736 | 12/1961 | Furst et al.     | 57/352 X  |
| 3,016,681 | 1/1962  | Andremont        | 57/354 X  |
| 3,022,025 | 2/1962  | Saxl             | 242/155   |
| 3,047,932 | 8/1962  | Pittman et al.   | 28/1      |
| 3,053,474 | 9/1962  | Luntz et al.     | 242/150 M |
| 3,095,630 | 7/1963  | Pittman          | 28/1      |
| 3,100,091 | 8/1963  | Mindheim et al.  | 242/150 M |

|           |         |                      |           |
|-----------|---------|----------------------|-----------|
| 3,106,442 | 10/1963 | Compostella et al.   | 18/48     |
| 3,112,600 | 12/1963 | Stoddard et al.      | 57/34     |
| 3,113,746 | 12/1963 | Steen                | 242/155   |
| 3,152,436 | 10/1964 | Dudzik et al.        | 57/157    |
| 3,194,000 | 7/1965  | Eldridge et al.      | 57/34     |
| 3,352,511 | 11/1967 | Wiggins              | 242/155   |
| 3,438,194 | 4/1969  | Cerutti et al.       | 57/157    |
| 3,457,715 | 7/1969  | Eldridge et al.      | 57/6      |
| 3,606,196 | 9/1971  | Heard                | 242/155 M |
| 3,724,409 | 4/1973  | Olney, Jr.           | 112/255   |
| 3,782,091 | 1/1974  | Spurgeon             | 57/34 HS  |
| 3,797,775 | 3/1974  | White                | 242/155 M |
| 3,831,880 | 8/1974  | White et al.         | 242/156   |
| 3,897,916 | 8/1975  | Rosen                | 242/155 M |
| 4,035,879 | 7/1977  | Schippers            | 28/246    |
| 4,112,561 | 9/1978  | Norris et al.        | 57/91 X   |
| 4,186,896 | 2/1980  | Brandenberger et al. | 242/131   |
| 4,313,578 | 2/1982  | Wilson et al.        | 242/150 M |

Primary Examiner—Donald Watkins

Attorney, Agent, or Firm—Earle R. Marden; H. William Petry

## [57] ABSTRACT

A direct current electromagnetic disc type tension control which periodically has the D. C. voltage increased from low voltage to high voltage and the high voltage is driven to zero a successive predetermined number of times to vibrate the tension discs in order to break the contact between the tension discs and between the tension discs and the electromagnet to lower the resistance to rotation of the discs.

6 Claims, 7 Drawing Figures





FIG. - 1 -



FIG. - 2 -



FIG. - 3 -

FIG. - 4 -



FIG. - 5 -



*FIG. - 7 -*



*FIG. - 6 -*

## D. C. YARN TENSION CONTROL

This invention relates generally to the employment of an electromagnetically actuated disc tension control to intermittently grasp and release a continuous filament synthetic yarn which is being processed downstream of the tension control.

It is an object of the invention to provide a yarn processing system which employs a disc tension control to randomly vary the tension of a yarn being processed in a yarn processing machine.

Other objects and advantages of the invention will become readily apparent as the specification proceeds to describe the invention with reference to the accompanying drawings, in which:

FIG. 1 is an overall schematic representation of the new and novel system to produce a textured, continuous filament synthetic yarn;

FIG. 2 is a partial perspective view of the yarn supply creel for the system shown in FIG. 1;

FIG. 3 is an exploded schematic view of the yarn tension disc device used in the system of FIG. 1;

FIG. 4 is a top view of the post of the yarn tension disc device of FIG. 3;

FIG. 5 is a side elevation view of the post shown in FIG. 4;

FIG. 6 is a schematic representation of the voltage control scheme for the yarn tension disc electromagnetic; and

FIG. 7 is a graphical representation of the voltage supplied to the electromagnet of the yarn tension disc device.

Looking now to FIG. 1, the overall system of FIG. 1 will be explained to obtain the novel disclosed yarn. The system is directed to a method to produce a specially textured yarn by intermittently varying the draw of a continuous filament partially oriented, synthetic, multifilament yarn such as polyester. The multifilament yarn 10 is supplied from a supply package 12 to the false twist device 14 by the feed roll device 16. The yarn 10 from the package 12 successively, in its travel to the feed roll device 16, passes through the balloon control apparatus 18, over the guide members 20, 22 and 24 through the electromagnetically controlled tension disc apparatus 26 and under the guide member 28 through the primary heater 30 and false twist device 14 to the feed roll device 16. The yarn 10 is intermittently and randomly drawn in the primary heater 30 by the intermittent hold back action of the disc tension apparatus 26. The discs 32 and 34 are intermittently and randomly drawn together and released on the yarn 10 by the action of the electromagnet 36 controlled by the varying voltage supplied thereto by a suitable voltage source which is varied by the action of a random signal generator.

From the feed roll device 16 the textured yarn passes through the secondary heater 37 with very little overfeed since the speed of the feed roll device 38 is substantially the same as the feed roll device 16 and the crimp in the yarn is allowed to set. Depending on the amount of crimp contraction desired the secondary heater can be turned on at an appropriate temperature or off or bypassed and the overfeed varied from high to very little.

The feed roll device 38 is driven at a higher speed than the feed roll device 44 to overfeed the textured yarn through the air jet entangling device 40 to com-

2  
mingle and entangle the individual filaments of the textured yarn. From the feed roll device 38 the entangled, textured yarn is slightly overfed to the yarn take-up package 42 by the feed roll device 44.

5 Schematically in FIG. 1, the yarn package 12 and the balloon control element 18 are shown as separate items but in actual practice a creel unit, designated 46 in FIG. 2, is used. The creel unit 46 supports a plurality of packages 12 for a plurality of false twist spindle positions and is slid in and out of position relative to a multiple spindle false twisting machine. In FIG. 2 a partial creel is shown supporting a pair of supply packages held on creel pins supported by creel pin support members 48 that are connected to the creel. Also connected to the creel is a horizontal separation plate 50 through which the yarn guide supports 52 project. A yarn guide 54 for each yarn package is connected thereto to guide the yarn 10 from the package 12 towards the guide member 20. Mounted on both sides of the horizontal separator plate 50 is a channel beam 56 between which is connected the balloon control apparatus or bar 18. The balloon of yarn from the creel is unusually erratic and violent due to the alternating take-off velocity and is therefore prone to entanglement if not controlled. As shown in FIG. 2 the bar 18 prevents yarn 10 from the package 12 from forming a full balloon and getting entangled in and around various elements of the creel such as yarn guides 54. As shown in FIG. 2, a second bar 18 is shown which is used for the same purpose for 10 the yarn packages (not shown) on the opposite side of the creel unit 46.

15 FIGS. 3-5 show the electromagnetically controlled tension disc apparatus 26 in detail. The apparatus 26 basically consists of the electromagnet 36, the spring biasing member 60 of Teflon or other suitable material, the tension discs 32 and 34, the disc post 62 and the screw 63 to maintain the aforementioned element in operative relationship. The disc 32 is made from a magnetically attractive material such as a ferrous material 20 while the disc 34 is manufactured from a non-magnetically attractive material. For reasons hereinafter explained the post 62 has a slot 64 therein which is offset from the centerline of the post. Also for reasons herein-after explained, it is desired to supply random, intermittent pulses of low and high D. C. voltage to cause the discs 32 and 34 to close randomly and intermittently and to cause the discs to vibrate relative to one another and relative to the electromagnet 36. To accomplish this action the arrangement shown in FIG. 6 is employed. 25 The random and intermittent supply of low and high D. C. pulses is caused by a random signal generator 66 of the type disclosed in U.S. Pat. No. 4,160,359 which indirectly affects the D. C. voltage supplied from the coil driver 68 to the coil 70 of the electromagnet 36. 30 Looking at FIGS. 6 and 7 together line 72 represents the condition when the random signal generator 66 is signaling the coil driver 68, through the computer 74 and the digital to analog connector 76, to supply a constant low voltage to the coil 70 to provide low tension on the yarn. Then randomly and intermittently the random signal generator 66 supplies a high tension pulse to the computer 76 and the AND gate 78 to cause the coil driver 68 to supply high D. C. voltage 80 to the coil. At the same time the high tension pulse is supplied 35 to the AND gate 78 to allow the 100 hertz oscillator 81, 50% duty cycle to provide an oscillating driver disabling signal 82 to the coil driver 68 to repeatedly drive the D. C. voltage to ground or zero 83 to provide the 40 45 50 55 60 65 70 75 80 85 90 95

square wave oscillation shown in FIG. 7. This action continues until the random signal generator 66 discontinues the high tension pulse and reverts to the supply of the low tension pulse to the computer 74. This repetitive action is represented graphically in FIG. 7 where the square wave portions are unequally spaced from one another by periods of low voltage or tension 72. As represented in FIG. 7 the rise and fall of the D. C. voltage is faster than A. C. voltage to provide rotation of the discs 32 and 34.

In FIG. 7 the lines 72 represent periods of low D. C. voltage on the coil 70 to provide low tension on the yarn between the discs 32 and 34 while 80 represents periods of high voltage on the coil 70 to cause the discs 32 and 34 to highly tension the yarn. Then the rapid fluctuations between 80 and 83 cause the discs to vibrate and allow rotation by the torque of the yarn passing through the slot 64 of the post 62. The vibration of the discs allows the discs to be rotated more easily so that the yarn passing through will subsequently clean out the finish deposited between the discs by the yarn.

Alternatively, the wall 84 defining one portion of the slot 64 can be eliminated and replaced by an upstanding guide member, not shown, which will serve to confine the yarn path to a path offset from the centerline of the post 62.

In the preferred form of the invention the spring biasing member 60 is of a diameter greater than the inner, internal diameter 85 and less than the inner, external diameter 86 of the lower tension disc 34 so that it is curved downward at its extremities when the discs 32 and 34 are pulled towards the electromagnet 36. Conversely, when the voltage to the electromagnet is reduced, the upward force exerted due to the bias of the member 60 urges the discs upward.

As described briefly before, it is desired to cause the tension discs 32 and 34 to rotate in order to dissipate the finish deposited therebetween by the yarn 10. As described above, the discs 32 and 34 are free to rotate on the post 62. To further enhance this rotation, the slot 64 is located off center of the centerline of the post so that the yarn passing between the discs 32 and 34 will exert a torque thereon. Furthermore, since yarn 10 is located in the slot 64 between the discs 32 and 34, the yarn cannot jump out from between the discs and have to be rethreaded. Further, such location of the yarn in the slot prevents uncontrolled texturing and lessens the tendency for yarn breaks.

In the form described hereinabove the preparation of a single end of multifilament synthetic yarn is described but, depending on the ultimate use of the yarn produced, a plurality of yarns can be interlaced or commingled in the air jet 40. Examples of such yarn are set forth below.

#### EXAMPLE 1

Two ends of a 240 denier, 68 filament DuPont 56T polyester yarn were processed as described above and entangled or interlaced in the air jet 40 to provide a 2/150/68 yarn with an actual denier of 321. The elongation was 51% with a crimp contraction of 1%. The operating conditions were as follows:

|                                         |           |
|-----------------------------------------|-----------|
| False Twist Spindle Speed               | 96000 RPM |
| Yarn Speed through Spindle yards/minute | 117       |
| False Twist turns/inch                  | 23        |
| Twist Multiple                          | 306       |
| Direction                               | "S"       |

-continued

|                                  |           |
|----------------------------------|-----------|
| Yarn Overfeed Through Heater 37  | By-passed |
| Yarn Overfeed Through Air Jet    | 4.0%      |
| Yarn Overfeed to Take-Up         | 1.7%      |
| Temperature of Heater 30         | 180° C.   |
| Temperature of Heater 37         | Off       |
| High Pre-Spindle Tension Average | 50 grams  |
| Low Pre-Spindle Tension Average  | 12 grams  |

10 The yarn thus produced has a very low crimp contraction with high luster and intermittent character.

#### EXAMPLE 2

15 Two ends of a 220 denier, 54 filament DuPont 693T polyester yarn were processed and entangled in the air jet 40 to provide a 2/150/54 yarn with an actual diameter of 328 denier. The elongation was 48% with a crimp contraction of 1.8%. The operating conditions were as follows:

|                                         |            |
|-----------------------------------------|------------|
| False Twist Spindle Speed               | 129000 RPM |
| Yarn Speed through Spindle yards/minute | 128        |
| False Twist turns/inch                  | 28         |
| Twist Multiple                          | 359        |
| Direction                               | "S"        |
| Yarn Overfeed Through Heater 37         | 0          |
| Yarn Overfeed Through Air Jet           | 4.0%       |
| Yarn Overfeed to Take-Up                | 1.7%       |
| Temperature of Heater 30                | 180° C.    |
| Temperature of Heater 37                | 190° C.    |
| High Pre-Spindle Tension Average        | 50 grams   |
| Low Pre-Spindle Tension Average         | 16 grams   |

The yarn produced has a low crimp contraction with very high luster and intermittent character.

35 It can readily be seen that the described apparatus and method provides a randomly, intermittently textured, continuous multifilament synthetic yarn which along its length has variable molecular orientation, bulk, torque, twist and shrinkage. The produced yarn has a 40 low crimp contraction and a high luster. This yarn is especially useful in the fabrication of a velvet-type upholstery fabric and provides unique visual effects due to its variable dye affinity.

45 Although the preferred embodiment of the invention has been described, it is contemplated that many changes may be made without departing from the scope or spirit of the invention and it is desired that the invention by only limited by the scope of the claims.

I claim:

50 1. Apparatus to produce a yarn having areas of differential bulk throughout its length comprising: a texturing device, supply means supplying continuous filament, synthetic yarn to said texturing device, a heater means located between said texturing device and said supply means to heat the yarn passing to said texturing device, means taking up yarn from said texturing device and a disc tension device mounted between said supply means and said heater means to vary the supply of yarn to said heater means, said disc tension including an electromagnet, a post member operably associated with said electromagnet, a first metallic disc member mounted on said post, a second metallic disc member mounted on said post adjacent said first disc member, means supplying direct current voltage to said electromagnet, said means 55 to supply direct current voltage including a first means to randomly and intermittently increase the direct current voltage to said electromagnet and a second means to drive the increased direct current voltage to substan-

tially zero to cause said first and said second disc members to move suddenly relative to one another.

2. The apparatus of claim 1 wherein said second means includes a means to periodically disable said means to supply direct current voltage.

3. An electromagnetically actuated tension device comprising: an electromagnet, a post member operably associated with said electromagnet, a first metallic disc member mounted on said post, a second metallic disc member mounted on said post adjacent said first disc member, means supplying direct current voltage to said electromagnet, said means to supply direct current voltage including a first means to randomly and intermittently increase the direct current voltage to said electromagnet and a second means to drive the increased direct current voltage to substantially zero to cause said first and said second disc members to move suddenly relative to one another.

4. The apparatus of claim 3 wherein said second means includes a means to periodically disable said mean to supply direct current voltage.

5. A method to produce a textured, continuous filament, synthetic yarn comprising the steps of: supplying a continuous filament, synthetic yarn from a supply package through an electromagnetically actuated disc tension device and a heater to a texturing device, supplying a low voltage direct current to the coil of the tension device, randomly and intermittently increasing the direct current voltage to the coil of the tension device, causing the discs of the tension device to vibrate by periodically driving the increased direct current voltage substantially to zero, texturing the synthetic yarn and taking up the textured yarn.

6. The method of claim 5 wherein the yarn is false twist textured.

\* \* \* \* \*

20

25

30

35

40

45

50

55

60

65